

# United States Patent [19]

Sonnenstine et al.

[11]

4,277,551

[45]

Jul. 7, 1981

[54] ELECTROPHOTOGRAPHIC PLATE  
HAVING CHARGE TRANSPORT  
OVERLAYER

[75] Inventors: Terry J. Sonnenstine, White Bear  
Lake; Kenneth G. Kneipp,  
Maplewood, both of Minn.

[73] Assignee: Minnesota Mining and  
Manufacturing Company, St. Paul,  
Minn.

[21] Appl. No.: 67,883

[22] Filed: Aug. 20, 1979

[51] Int. Cl.<sup>3</sup> ..... G03G 13/14; G03G 5/04;  
G03B 21/00

[52] U.S. Cl. ..... 430/120; 430/48;  
430/58; 430/59; 430/84; 430/85; 430/86;  
430/95; 430/128; 355/3 DD; 355/3 CH

[58] Field of Search ..... 430/58, 59, 85, 95,  
430/84, 86, 120, 48, 128, 31; 355/3 DD, 3 CH

## [56] References Cited

### U.S. PATENT DOCUMENTS

2,901,348 8/1959 Dessauer ..... 430/67

|           |         |                      |        |
|-----------|---------|----------------------|--------|
| 3,723,105 | 5/1973  | Kitajima et al. .... | 430/85 |
| 3,791,826 | 2/1974  | Cherry .....         | 430/58 |
| 3,879,199 | 4/1975  | Trubisky et al. .... | 430/58 |
| 3,928,034 | 12/1975 | Regensburger ....    | 430/58 |
| 4,088,484 | 5/1978  | Okazaki et al. ....  | 430/58 |
| 4,115,116 | 9/1978  | Stolka et al. ....   | 430/58 |
| 4,121,981 | 10/1978 | Ward et al. ....     | 430/85 |

Primary Examiner—Richard L. Schilling  
Attorney, Agent, or Firm—Cruzan Alexander; Donald  
M. Sell; William B. Barte

## [57] ABSTRACT

An electrophotographic plate comprising a conductive substrate, a photoconductive-insulative layer overlaying the substrate and a transparent, electrically active, organic, electron transport layer overlaying the photoconductive-insulative layer in which the photoconductive layer comprises a Se—Te or Se—As mixture in the range of 90–97.5 atomic percent Se or 60–97.5 atomic percent, respectively, and wherein the thicknesses of the photoconductive layer and transport overlayer range between 40 to 100 micrometers and 1 to 5 micrometers, respectively.

14 Claims, 5 Drawing Figures





FIG. 1



FIG. 2



FIG. 3



FIG. 4



FIG. 5

## ELECTROPHOTOGRAPHIC PLATE HAVING CHARGE TRANSPORT OVERLAYER

### FIELD OF THE INVENTION

This invention relates to electrophotography and in particular to xerographic plates, drums, etc. on which an electrostatic image may be produced and which includes a conductive substrate, a photoconductive layer, and a charge transport overlayer.

### DESCRIPTION OF THE PRIOR ART

In the art of electrophotography, and particularly xerography, it is well known to provide a photoconductive xerographic article such as a plate or drum, by coating a conductive substrate, such as an electrically conductive aluminum drum, with a photoconductive-insulative layer to form a composite layered photosensitive article. The surface of the layered article is then uniformly electrostatically charged and exposed to a pattern of activating electromagnetic radiation, such as light. Charge is selectively dissipated in the illuminated areas of the photoconductive-insulative layer, thus leaving an electrostatic charge image in the non-illuminated areas. The electrostatic charge image can then be developed to form a visible image if desired. The developed image may be fixed or made permanent on the photoconductive-insulative surface, or may be transferred to paper or some other material, and subsequently affixed by some suitable means.

The conductive substrate utilized in such electrophotographic articles usually comprises a metal such as brass, aluminum, gold, platinum, steel or the like, and may be of any convenient thickness, rigid or flexible, and in the form of a sheet, web or cylinder. The substrate may also comprise other materials such as metallized paper and plastic sheets or glass coated with a thin conductive coating. In all cases it is usually preferred that the substrate be strong enough to permit a certain amount of handling.

Typical photoconductive-insulative materials useful in forming xerographic articles include: (1) inorganic crystalline photoconductors such as cadmium sulfide, cadmium sulfoselenide, cadmium selenide, zinc sulfide, zinc oxide, and mixtures thereof, (2) inorganic photoconductive glasses such as amorphous selenium, selenium alloys, and selenium-arsenic, and (3) organic photoconductors such as phthalocyanine pigments and polyvinyl carbazole with or without additive materials which extend its spectral sensitivity.

During operation in a typical electrophotographic copying machine, the photoconductive surface of the xerographic article is exposed to the surrounding environment, and as such, is susceptible to abrasion, chemical attack, heat, and multiple exposures to light during cycling. Such exposures produce a gradual deterioration in the electrical characteristics of the photoconductive-insulative layer, resulting in defects or marks in the resultant copies which correspond to surface defects and scratches and to localized areas of persistent conductivity on the surface which fail to retain an electrical charge and high dark discharge. In addition, in order to provide the requisite photoconductive and insulative properties, it has generally been found necessary that the photoconductive-insulative layer comprise either 100% of the layer, as in the case of vitreous selenium, or that it contain a high proportion of photoconductive particles in a binder. This requirement restricts the

physical characteristics, such as flexibility and adhesion of the photoconductor, of the final article, be it a plate, drum or belt, in that the characteristics are predominantly controlled by the photoconductive material and not by the resin or matrix material which is preferably present in a minor amount.

In such conventional electrophotographic articles, upon exposure to light the photoconductive properties of the photoconductive-insulative layer result in charge transport through the bulk of the layer in the case of homogeneous constructions, or through the highly loaded photoconductive particles in the case of particle-binder constructions to thereby selectively dissipate an electrostatic charge on the surface. In order to improve the physical characteristics of the outer surface to lessen the impact of environmental effects while also allowing the transport of photogenerated charge carriers to the surface, it is also known to provide a multilayered xerographic article in which a photoconductive layer on a conductive substrate is, in turn, covered by an organic insulating layer. Such structures are, for example, depicted in U.S. Pat. Nos. 2,901,348 (Dessauer et al), 3,837,851 (Shattuck et al), 3,791,826 (Cherry et al) and 3,928,034 (Regensburger).

U.S. Pat. No. 2,901,348 (Dessauer et al) depicts a multilayered electrographic article comprising in sequence, a conductive substrate, an insulating barrier layer, a p-type photoconductive-insulator layer, preferably of vitreous selenium having a thickness in the range of 20-50  $\mu\text{m}$ , and an outer, very thin, insulative charge acceptor layer. Since the outer layer is said to be preferably less than one  $\mu\text{m}$  thick and usually on the order of 50-500 nm, the ratio of the top coat to photoconductive layer may be in the range of 0.04 to 1. Other than a general description of various insulating waxes and resins, no particularly preferred top-coat material is suggested, either chemically or in terms of desired electrical or physical properties. Such thick selenium layers are undesirable in that excessive residual charge buildup is encountered during cyclical operations.

In contrast to the ratios of top coat to photoconductor layer apparently present in the examples depicted in Dessauer et al, the remaining patents noted above are directed to multilayered articles in which the overlaying charge transport layer is typically thicker than the photoconductive-insulative layer. Such a construction is said to be desired in order that the photoconductive layer be sufficiently thin to avoid residual charge buildup and to enable the electrographic article to be flexible. Thus, for example, in U.S. Pat. No. 3,791,826 (Cherry et al) an electrophotographic plate is depicted which comprises a conductive substrate, a barrier layer, an inorganic charge generating layer, and an organic charge transport overlayer. In that patent, the charge generating layer is required to be at least 0.15  $\mu\text{m}$  thick in order to allow the generation of sufficient charge, and that it is generally preferable to be less than about one micrometer. The organic charge transport layer is required to be between 3 and 20 micrometers thick, it being indicated that layers thinner than 3  $\mu\text{m}$  will not accept sufficient voltage to be useful. Thicker layers are said to provide a high resistivity surface which can support an electronic charge on the surface, while also transporting electronic charge from the charge generating layer. The charge transport layer is there disclosed to preferably comprise at least about 20 weight % of the compound 2,4,7-trinitro-9-fluorenone (TNF), which is

further preferably combined with a polyethylene terephthalate resin binder.

U.S. Pat. No. 3,837,851 (Shattuck et al) is relevant to the present invention in that it depicts a multilayered electrophotographic article in which a charge transport layer, here based on triarylpyrazoline, is placed adjacent a charge generation layer. Particularly, in an example closest to the present invention, the article is said to consist of a charge generating layer of 68% Se, 30% Te, and 2% As, evaporated onto a barrier coated conductive substrate which is in turn coated with a 15  $\mu\text{m}$  layer of a pyrazoline compound. The thickness of the charge generating layer is believed to be approximately 0.3  $\mu\text{m}$ .

U.S. Pat. No. 3,928,034 (Regensburger) describes an electrophotographic article which includes a photoconductive layer in which electron-hole pairs are generated, such as amorphous selenium, and an overlapping layer of an electrically active transport material into which the appropriate charge carrier may be injected. The electrically active transport material is characterized as being substantially transparent and non-absorbing in the particular wavelength region of xerographic use. Even though the described article appears to overcome some of the problems present in earlier xerographic articles, it too has its shortcomings. To prevent undesirable residual buildup of positive charges in the photoconductive layer during recycling, and to prevent excessive dark decay, Regensburger discloses that the photoconductive layer be less than 20  $\mu\text{m}$  thick, and preferably be around 1  $\mu\text{m}$ . Conversely, the overlaying layer of electrically active transport material is recited to be quite thick, on the order of 10 to 20  $\mu\text{m}$ , such that sufficient amounts of electrostatic charge can be accepted. A device so constructed is characterized by residual charge buildup during operation, causing excessive backgrounding, or alternatively, a slow recycling rate. In addition, even though the overlayer is substantially transparent, as thicker layers are required, absorption and scattering due to included particles and partial crystallization become significant and have a detrimental effect upon the sensitivity of the device and the quality of copies produced.

#### SUMMARY OF THE INVENTION

Akin to electrophotographic articles disclosed in the prior art, such as those discussed hereinabove, the present invention is also directed to an electrophotographic article comprising a conductive substrate, a photoconductive-insulative layer overlaying the substrate and a transparent electrically active organic electron transport layer overlaying the photoconductive-insulative layer. However, in contrast to such articles of the prior art, the article of the present invention comprises a relatively thick photoconductive-insulative layer and a relatively thin electron transport layer adjacent thereto, in which the photoconductive-insulative layer comprises vitreous selenium and a material selected from the group consisting of tellurium and alloys thereof in which selenium is present in an amount within the range of 90 and 97.5 atomic percent. Specifically, the photoconductive-insulative layer of the article of the present invention has a thickness within the range between 40 and 100 micrometers, while the electron transport layer has a thickness within the range between 1-5 micrometers, such that the ratio of the thickness of the transport layer to that of the photoconductive-insulative layer is between 1:8 and 1:100.

In contrast to the articles depicted in the prior art or those suggested thereby, it has now been found that selenium-tellurium compositions in the range of 90:10 to 97.5:2.5 (preferably 95:5) allow the use of an exceedingly thick photoconductive-insulative layer (40-100  $\mu\text{m}$ ) overcoated with a very thin (1-5  $\mu\text{m}$  thick) layer of an electron charge transport material. In a particularly preferred embodiment, the layer of transport material comprises 2,4,7-trinitro-9-fluorenone (TNF) dissolved in an organic binder such as a thermoplastic polycarbonate condensation product of bisphenol-A and phosgene. Such a construction has been found to exhibit very large charge acceptance and to retain low residual charge in light struck areas even after repeated cycling. Thus, there is virtually no background in the developed images and excellent copies are therefore produced. The overcoated charge transport layer is also easily cleaned, reduces the rate of drum aging, and protects against scratching from toner abrasion and paper jams.

#### BRIEF DESCRIPTION OF THE DRAWING

FIG. 1 is a cross section of an exemplary electrophotographic device pursuant to the present invention;

FIGS. 2 and 3 are cross sections of a device similar to that shown in FIG. 1 showing the manner in which charges are generated and dissipated during the use of such a device;

FIG. 4 is a cross section of an exemplary prior art device, and

FIG. 5 is a graph showing the effect on certain electrical properties of the top coating layer pursuant to the present invention.

#### DESCRIPTION OF THE PREFERRED EMBODIMENTS

An exemplary embodiment of the present invention is shown in FIG. 1 where in cross section it may be seen that the electrophotographic device 10 includes a conductive substrate 12 onto which is coated a photoconductive-insulative layer 14 and in turn on top of which is placed an overcoat of an electron transport layer. The thickness of the photoconductive-insulative layer 14 is maintained in the range of 40 to 100 micrometers, while that of the electron transport layer is maintained to have a thickness in the range between 1 and 5 micrometers.

The substrate 12, in addition to being electrically conductive, is desirably also capable of lending physical support to the overall structure. It may be comprised of a metallic sheet such as an aluminum drum blank or the like, or be a composite metal coating on a sufficiently rigid dielectric substrate. The metal may similarly be selected from materials such as brass, aluminum, steel or the like. Further, while the overall configuration of the structure is typically provided in a drum form so as to be utilizable in a copy machine in which the drum rotates about a graphic original, the plates may similarly be used in a flat format or otherwise as desired.

The photoconductive-insulative layer 14, as mentioned above, is provided in a thickness ranging between 40 and 100 microns and is produced by vacuum evaporation of alloys of selenium together with tellurium. In the event a selenium/tellurium alloy is desired, the ratio of selenium is selected to be within the range of 90 and 97.5 atomic percent, and preferably should be 95% Se and 5% Te. Contrary to prior art teachings such as discussed hereinabove, it has been found that compositions within the range of 90 to 97.5 atomic percent selenium allow the use of thick photoconduc-

tive insulative films in the range of 40 to 100 micrometers, in combination with a very thin overcoat electron transport layer 16. Particularly, if the charge transport layer 16 is selected to be 2,4,7-trinitro-9-fluorenone (TNF) dissolved in polycarbonate binder such as General Electric Lexan® brand Type 145, the thickness of the overcoat need only be in the range of 1 to 5 micrometers and preferably about 2 micrometers when used together with a photoconductive-insulative layer of about 65 micrometers.

The electron transport layer 16 is preferably prepared by dip coating a suitably prepared photoconductive-insulative coated drum in a solution containing solids such that about 70 weight percent of the solids is a binder such as General Electric Lexan® brand polycarbonate Type 145 and 30 weight percent of the solids is TNF. End to end uniformity of such a dip coated layer is achieved by employing low viscosity solutions for dipping where the rate of flow of the solution across the face of the drum is greater than the rate of drying. It has generally been found that the transport layer 16 desirably comprises aromatic or heterocyclic electron acceptor materials which have been found to exhibit negative charge carrier transport properties, as well as requisite transparency characteristics. Typical electron acceptor materials within the purview of the instant invention include phthalic anhydride, tetrachlorophthalic anhydride, benzil, mellitic anhydride, S-tricyanobenzene, picryl chloride, 2,4-dinitrochlorobenzene, 2,4-dinitrobromobenzene, 4-nitrobiphenyl, 4,4-dinitrobiphenyl, 2,4,6-trinitroanisole, trichlorotrinitrobenzene, trinitro-o-toluene, 4,6-dichloro-1,3-dinitrobenzene, 4,6-dibromo-1,3-dinitrobenzene, p-dinitrobenzene, chloranil, bromanil, and mixtures thereof. It is further intended to include within the scope of those materials suitable for the active transport layer, other reasonable structural or chemical modifications of the above described materials provided that the modified compound exhibits the desired charge carrier transport characteristics.

While any and all aromatic or heterocyclic electron acceptors having the requisite transparency characteristic are within the purview of the instant invention, particularly good electron transport properties are found with aromatic or heterocyclic compounds having more than one substituent of the strong electron withdrawing components such as nitro(-NO<sub>2</sub>), sulfonate ion (-SO<sub>3</sub>), carboxyl (-COOH) and cyano(-CN) groupings. From this class of materials, 2,4,7-trinitro-9-fluorenone (TNF), 2,4,5,7-tetrinitrofluorenone, trinitroanthracene, dinitroacridine, tetracyanopyrene, and dinitroanthraquinone are preferred materials because of their availability and superior electron transport properties.

Similarly, while a polycarbonate binder such as General Electric Lexan is primarily desired, other binder materials such as polystyrene, silicone resins such as DC-801, DC-804, and DC-996 manufactured by Dow Corning Corporation, acrylic and methacrylic ester polymers such as Acryloid A-10 and Acryloid B-72, polymerized ester derivatives of acrylic and alpha-acrylic acids such as supplied by Rohm & Haas Company, and polymerized butyl methacrylates such as Lucite 44, Lucite 45 and Lucite 46 supplied by E. I. duPont DeNemours & Company, as well as fluorinated rubbers, vinyl polymers and copolymers, cellulose esters, etc., may similarly be utilized.

To sensitize the electrophotographic device shown in FIG. 1 to imaging radiation, the structure is connected as shown in FIG. 2 with the conductive substrate connected to ground and the top layer 16 charged in the dark with a positive corona. The resultant positive charge layer has associated therewith a proportionate negative charge on the grounded substrate 12. Optimum behavior of such a sensitized device is found to result if the photoconductive-insulative layer 14 is sufficiently

10 resistive under dark conditions so as not to dissipate the applied electrical charge prior to completion of the imaging procedure. Other conditions desirable for optimum behavior include a relationship between the photoconductive-insulative layer 14 and the overcoat layer 16, such that the combination can accept a high 15 electrical field without electrical breakdown or charge conduction, and further that the photoconductive insulative layer 14 be an efficient injector of electrons into the top coat 16 and of holes into the conductive substrate 12.

As further shown in FIG. 3, such a sensitized device 20 may then be imaged by directing light onto the transport layer 16. The light passes through the layer 16 and is absorbed by the photoconductive-insulative layer 14, 25 creating electron hole pairs 18. The electrons and holes are separated under the electric field resulting from the retained charges. The electrons are injected into and transported through the electron transport layer 16 while the holes are transported through the photoconductive-insulator 14, thereby imagewise discharging the surface charges where light strike, in proportion to the integrated amount of light being absorbed. In regions where radiation does not impinge upon the device, the charge distribution remains substantially the same as 30 prior to the imaging. The imaging step is now complete, an electrostatic charge image having been formed on the surface. The image may then be developed with toners in a conventional manner to form a toner image on the surface of the drum.

40 Because of the novel construction of the electrophotographic device of the present invention, a very low residual charge remains in areas where light impinges upon it, thereby resulting in virtually no background in the toner image. This behavior is evidenced in excellent copy quality were the copies are made by transferring the toner image to plain paper, particularly when repeated charging and imaging operations are experienced. Added permanence is introduced in the transferred toner image when the heat fusion or pressure 45 fusion steps are added. The topcoat surface is subsequently easily discharged and cleaned by conventional techniques.

To illustrate the contrast between the present invention and that of a prior art device wherein a similar 55 selenium drum would be provided, and using the relative thicknesses of the drum and topcoat as taught in the prior art, such a device would have a configuration as shown in FIG. 4. In such a case, the device 20 would include a conductive substrate 22 on which a photoconductive-insulative layer 24, nominally having a thickness of about 1 or 2 microns or less and in all cases less than about 20 microns, would have overcoated thereon a thick electron transport layer 26. As was mentioned hereinabove, thin photoconductive insulative layers such as the layer 24, were previously required to avoid producing undesirable positive residual charge build-up in the photoconductive insulative layer. Because of 60 such a requirement, the overlying electron transport 65

layer 26 was necessarily thick, such as in the 10 to 20 micrometer range, in order to attain a desirable amount of charge acceptance across the device. The thick topcoat then itself causes a large and undesirable residual charge build-up. Alternatively, if such a thick topcoat was sufficiently heavily loaded with an electron charge transporting component such as TNF, the component tended to crystallize out, thus producing a rough surface which provides traps for toner powder. Such traps prevent ready cleaning of the surface following each exposure and result in black spots on the subsequent copies.

#### EXAMPLE 1

A specific embodiment of the device dimensioned as shown in FIG. 1 was prepared as follows: An aluminum drum was provided with a chemically clean surface, onto which was vacuum evaporated a layer of selenium tellurium alloy having a ratio of 95:5 atomic percent selenium to tellurium. A layer approximately 60 micrometers was thus provided. The selenium tellurium coating was then in turn dip coated in a solution of 2,4,7-trinitro-9-fluorenone (TNF) and Lexan® to produce a layer approximately 2 micrometers thick when dry. The solution used for producing the TNF/LEXAN® overcoat was prepared as follows:

| Ingredients                       | Wt. in Grams | % Wt. of Total |
|-----------------------------------|--------------|----------------|
| Dichloromethane                   | 480          | 47.2           |
| 1,2-Dichloroethane                | 480          | 47.2           |
| GE Lexan® Type 145                | 40           | 3.9            |
| 2,4,7-trinitro-9-fluorenone (TNF) | 17.15        | 1.7            |

Upon drying, the dichloromethane and dichloroethane evaporate, leaving a layer consisting of approximately 70 wt.% Lexan® 145 and 30 wt.% TNF.

The topcoat is preferably provided by mounting the selenium-tellurium coated drum on a vertical rod and using a motor drive to control the rate of vertical motion, slowly withdrawing the drum from the coating solution at a rate of approximately 1 centimeter per second. While the rate at which the solution thus flows across the surface of the drum continually varies during withdrawal due to the displacement of the solution by the drum, this variability in the rate of flow does not appear to cause any non-uniformity in the coating thickness. In order to provide a control so as to enable determination of the relative effectiveness of the overcoating, only the lower half of the drum was inserted into the coating solution thus providing a coating on one half of the drum, with the other half being left uncoated. The thus produced electrophotographic drum was then placed in a 3M Brand SECRETARY II copy machine, wherein excellent copies of an original document were produced, both from the coated as well as from the uncoated sides of the drum. However, the positive effect of the 2 micrometer thick Lexan®/TNF overcoating was demonstrated as follows. The surface potential on the drum after charging in a non-functional test apparatus was determined to be approximately 1150 volts on the top coated portion of the drum, while a surface potential of only approximately 1050 volts was developed on the uncoated portion. The drum was then utilized in the SECRETARY II machine and 1,000 copies made using the drum. To accelerate the rate of possible crystallization of the selenium tellurium layer, the drum was then heated at 65 degrees Centigrade for

6.5 hours. The surface potential was then again measured as in the same non-functional test apparatus and was found again to accept a charge of 1150 volts in the topcoated portion of the drum, whereas a potential of only 750 volts was attained on the non-topcoated portion. This reduction in surface potential on the non-topcoated portion was observed to be sufficient to cause a significant decrease in image density.

The effect of the topcoat on the crystallization of the Se-Te photoconductive-insulative layer in an electro-photographic drum as used in the 3M Brand SECRETARY II machine is shown in FIG. 5. In that Figure, capacitance is plotted as a function of the time of heating. It may be noted that the non-topcoated portion of the drum exhibited an increase in the capacitance as a function of heating time. Such an increase in capacitance is evidence of an increase in the dielectric constant of the photoconductive-insulative drum and is believed to be attributed to the increased crystallization in the layer. In contrast, essentially no change in the capacitance was observed for the topcoated portion of the drum, thus indicating that no change in the crystallization of the Se-Te layer resulted during the heating operation. It is believed that the topcoat thus seals the surface of the Se-Te layer and minimizes the occurrence of scratches and the like on the Se-Te layer such that nucleation sites and other defects which would promote crystallization during continued use are minimized.

#### EXAMPLE 2

To further show the effectiveness of the electron transport overlayer pursuant to the present invention, a second selenium-tellurium (95:5) coated aluminum drum was prepared as in Example 1. By appropriately masking the surface of the drum, one portion of the drum was spray coated with a solution containing 2 wt.% solids of Lexan® and TNF, together with equal portions of dichloromethane, and 1,2-dichloroethane, the ratio of Lexan® to TNF being approximately 70:30, so as to result in 30 wt.% of TNF in the final coating. The first portion of the drum was coated to provide a dry thickness of about 2 micrometers thick. The same solution was spray coated onto a second portion of the drum for an extended length of time to provide a dry coating thickness of about 5 micrometers, while a third section of the drum was left uncoated. Testing of the drum in a 3M Brand SECRETARY Type III copy machine indicated no significant differences in copy quality. Non-functional test data indicated only slight charge acceptance and residual potential differences among the three drum sections. Whereas the non-topcoated portion of the drum was found to accept a charge of approximately 975 volts, the 2 micrometer Lexan®/TNF coated portion accepted a charge of approximately 1035 volts and the 5 micrometer coated portion accepted a charge of approximately 1,030 volts. The residual voltage retained after approximately 50 cycles was found to be about 10 volts on the non-topcoated portion and 25 and 40 volts, respectively, on the two micrometer and 5 micrometer topcoated portion. Such residual charges on all three portions were found to be negligible and not to be associated with any significant decreases or changes in the copy quality.

## EXAMPLE 3

A Se-Te (95:5) coated aluminum drum was again prepared as in Example 1. Also, as in Example 1, in this example the drum was also dipcoated, but in 3 respective sections, employing TNF/Lexan® polycarbonate solutions. Generally, it was observed that dipcoating provided a smoother and more defect-free coating than the spray coating technique utilized in Example 2. In this Example, one portion of the drum was dipped into a two percent Lexan® polycarbonate solution containing 30 wt.% TNF in a 50:50 wt.% mixture of dichloromethane and 1,2-dichloroethane, while a second section of the drum was dipped into a similar 4% solution to provide a thicker Lexan®/TNF coating. The center portion of the drum was left with no topcoat. Coating thicknesses on one portion were estimated to be 0.5-1 micrometer thick and to be 1-2 micrometers thick on the other coated portion. Non-functional test data again indicated but slight differences along the three drum sections, and the testing of the drum in a 3M Brand SECRETARY III machine indicated no appreciable differences in copy quality. The non-functional test data indicated that the charge acceptance on the three portions of the drum were in the range between 960 to 990 20 volts. The residual voltage retained after 50 cycles was 5 volts along the non-topcoated portion and increased to 40 volts on the 1-2 micrometer TNF/Lexan® coated portion.

## EXAMPLE 4

To further demonstrate the utility of the electron acceptance material in the topcoat layer, a selenium-tellurium (95:5) coated drum was first prepared as in Example 3 and opposite ends of the drum were then dipcoated in sections employing an undoped Lexan® solution, i.e. with no TNF present, and in a TNF/Lexan® solution, respectively. The first section of the drum was dipped in a 6% Lexan® polycarbonate solution in a 50/50 wt.% mixture of dichloromethane and 1,2-dichloroethane. The opposite section of the drum was dipped into an identical solution in which 30 wt.% TNF was added. The center section of the drum was left uncoated. The coating thicknesses of both coated sections was estimated to be approximately 2 to 5 micrometers thick. The section of the drum with the Lexan® topcoat was found to be characterized by a very high residual potential, and also showed excessive backgrounding when tested in a 3M Brand SECRETARY III machine. Specifically, the section having a Lexan® only topcoat was found to accept a charge of approximately 1150 volts. However, after 50 cycles a residual potential of 990 volts was present. In contrast, the section of the drum with no topcoat was found to accept an initial charge of 1,085 volts and to have no residual charge, while the section containing a TNF/Lexan® topcoat was found to accept 1130 volts of charge and to exhibit a residual potential after 50 cycles of only 30 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 9775 9780 9785 9790 9795 9800 9805 9810 9815 9820 9825 9830 9835 9840 9845 9850 9855 9860 9865 9870 9875 9880 9885 9890 9895 9900 9905 9910 9915 9920 9925 9930 9935 9940 9945 9950 9955 9960 9965 9970 9975 9980 9985 9990 9995 10000 10005 10010 10015 10020 10025 10030 10035 10040 10045 10050 10055 10060 10065 10070 10075 10080 10085 10090 10095 10100 10105 10110 10115 10120 10125 10130 10135 10140 10145 10150 10155 10160 10165 10170 10175 10180 10185 10190 10195 10200 10205 10210 10215 10220 10225 10230 10235 10240 10245 10250 10255 10260 10265 10270 10275 10280 10285 10290 10295 10300 10305 10310 10315 10320 10325 10330 10335 10340 10345 10350 10355 10360 10365 10370 10375 10380 10385 10390 10395 10400 10405 10410 10415 10420 10425 10430 10435 10440 10445 10450 10455 10460 10465 10470 10475 10480 10485 10490 10495 10500 10505 10510 10515 10520 10525 10530 10535 10540 10545 10550 10555 10560 10565 10570 10575 10580 10585 10590 10595 10600 10605 10610 10615

that many modifications and variations are both conceivable and practicable. All such alternative modifications thus fall within the true spirit and scope of this invention.

Having thus described the present invention, what is claimed is:

1. An electrophotographic plate comprising a conductive substrate, a photoconductive-insulative layer overlaying the substrate and a transparent, electrically-active, organic, electron transport layer overlaying the photoconductive-insulative layer, characterized by the photoconductive-insulative layer comprising vitreous selenium and tellurium and alloys thereof, in which selenium is present in an amount within the range of 90 and 97.5 atomic percent, the photoconductive-insulative layer having a thickness within the range of 40-100  $\mu\text{m}$  and the electron transport layer having a thickness within the range of 1-5  $\mu\text{m}$  such that the ratio of the thickness of the electron transport layer to that of the photoconductive-insulative layer is between 1:8 and 1:100, and by said electron transport layer comprising not greater than 35 weight percent of an aromatic or heterocyclic organic electron acceptor material dispersed in an organic binder.

2. A plate according to claim 1, wherein said electron acceptor material is selected from the group consisting of 2,4,7-trinitro-9-fluorenone, 2,4,5,7-tetranitrofluorenone, trinitroacridine, tetracyanopyrrole, and dinitroanthraquinone.

3. A plate according to claim 2, wherein said binder comprises a thermoplastic polycarbonate condensation product of bisphenol-A and phosgene.

4. A plate according to claim 1, wherein said electron transport layer is approximately 3 to 4 micrometers thick.

5. A plate according to claim 1, wherein said photoconductive-insulator layer consists of approximately 95 atomic percent Se and 5 atomic percent tellurium.

6. A plate according to claim 1, wherein said photoconductive-insulator layer is approximately 65 micrometers thick.

7. A plate according to claim 1, further comprising an insulative barrier layer between the conductive substrate and the photoconductive-insulative layer.

#### 8. A method of imaging comprising

(a) providing an electrophotographic plate having a conductive substrate, a photoconductive-insulative layer overlaying the substrate, and an electron transport layer overlaying the photoconductive-insulative layer, the photoconductive-insulative layer comprising vitreous selenium and tellurium and alloys thereof, in which selenium is present in an amount within the range of 90 and 97.5 atomic percent and the electron transport layer comprising a coating of not greater than 35 weight percent of an aromatic or heterocyclic organic electron acceptor dispersed in an organic binder, the photoconductive insulative layer having a thickness within the range of 40-100  $\mu\text{m}$  and the electron transport layer having a thickness within the range of 1-5  $\mu\text{m}$  such that the ratio of the thickness of the thickness of the

5

10

15

20

25

30

35

40

45

50

55

60

65

electron transport layer to that of the photoconductive-insulative layer is between 1:8 and 1:100, (b) uniformly charging the plate to a predetermined positive potential, and

(c) exposing the plate to a source of radiation to which the transport layer is substantially transparent and to which the photoconductive-insulative layer is responsive to result in the photo-generation of electron-hole pairs such that said radiation passes through the transport layer and causes said electron-hole pairs to be generated, said electrons and holes then being transported to form a latent electrostatic charge image on the surface of the plate.

9. A method according to claim 8, wherein said providing step includes evaporating onto the substrate a composition consisting of selenium and tellurium wherein selenium is present in an amount within the range of 90 and 97.5 atomic percent.

10. A method according to claim 9, wherein said evaporating is selected to provide a layer consisting of 95 atomic percent selenium and 5 atomic percent tellurium.

11. A method according to claim 8, further comprising developing the latent image to make it visible.

12. A method according to claim 8, comprising applying a coating onto the photoconductive-insulative layer of a solution of 2,4,7-trinitro-9-fluorenone and a binder comprising a thermoplastic polycarbonate condensation product of bisphenol-A and phosgene in a solvent including dichloromethane and dichloroethane.

13. A system for forming electrographic images comprising

(a) an electrophotographic plate including a conductive substrate, a photoconductive-insulative layer overlaying the substrate, and a transparent, electronically-active, organic, electron transport layer overlaying the photoconductive-insulative layer characterized by

the photoconductive-insulative layer comprising vitreous selenium and tellurium and alloys thereof, in which selenium is present in an amount within the range of 90 and 97.5 atomic percent, the photoconductive-insulative layer having a thickness within the range of 40-100  $\mu\text{m}$  and the electron transport layer having a thickness within the range of 1-5  $\mu\text{m}$  such that the ratio of the thickness of the electron transport layer to that of the photoconductive-insulative layer is between 1:8 and 1:100,

(b) means for uniformly charging the plate to a predetermined positive potential, and

(c) means for exposing the plate to a source of radiation to which the transport layer is substantially transparent and to which the photoconductive-insulative layer is responsive to result in the photo-generation of electron-hole pairs such that said radiation passes through the transport layer and causes said electron-hole pairs to be generated, said electrons and holes being transported to form a latent electrostatic charge image on the surface of the plate.

14. A system according to claim 13, further comprising means for developing the latent image to make it visible.

\* \* \* \* \*